# EUROPEAN PATENT SPECIFICATION

(11) **EP 0 416 131 B1**
(45) Date of publication and mention of the grant of the patent: **19.10.1994**
(21) Application number: 90904938.9
(22) Date of filing: 26.03.1990
(51) Int. Cl.: H01B 7/02, H01B 3/12, H01B 7/34, H01B 13/16, C25D 11/38, C23C 28/04

(54) **INSULATED ELECTRIC WIRE**
ISOLIERTE ELEKTRISCHE LITZE
FIL ELECTRIQUE ISOLE

(30) Priority: 28.03.1989 JP 77028/89; 20.03.1990 JP 70843/90
(43) Date of publication of application: 13.03.1991
(73) Proprietor: SUMITOMO ELECTRIC INDUSTRIES, LTD., Osaka-shi, Osaka 541 (JP)
(72) Inventor: INAZAWA, Shinji, c/o Osaka Works of Sumitomo, Kohana-ku, Osaka-shi, Osaka 554 (JP); YAMADA, Kouichi, c/o Osaka Works of Sumitomo, Konohana-ku, Osaka-shi, Osaka 554 (JP); SAWADA, Kazuo, c/o Osaka Works of Sumitomo, Konohana-ku, Osaka-shi, Osaka 554 (JP)
(74) Representative: Kirschner, Klaus Dieter, Dipl.-Phys.
(86) International application number: JP9000401
(87) International publication number: WO9011603

(56) References cited:
- EP-A- 0 292 780

## Description

### SPECIFICATION

### Field of the Invention

The present invention relates to an insulated wire, and more particularly, it relates to an insulated wire such as a distribution wire, a wire for winding or the like which is employed under high-vacuum environment or high-temperature environment such as a high-vacuum apparatus or a high-temperature service apparatus.

### Background of the Invention

An insulated wire may be applied to equipment such as heating equipment or a fire alarm, for which safety under a high temperature is required. Further, the insulated wire is also used under environment in an automobile, which is heated to a high temperature. An insulated wire formed by a conductor which is coated with heat resistant organic resin such as polyimide, fluorocarbon resin or the like has generally been used as such an insulated wire.

As to application for which high heat resistance is required, or employment under environment for which a high degree of vacuum is required, organic coating is insufficient in view of heat resistance, no gas emission property and the like. Thus, an insulated wire of such a form that a conductor is inserted in an insulator tube of ceramics, an MI cable (Mineral Insulated cable) of such a form that a conductor is inserted in a heat resistant alloy tube of a stainless steel alloy etc. which is filled with metal oxide powder of magnesium oxide etc., or the like has been employed for such application.

A fiber-glass braided insulated wire employing textile glass fiber as an insulating member etc. is listed as an insulated wire for which flexibility is required with heat resistance.

In the aforementioned insulated wire coated with organic resin having heat resistance, the highest temperature at which insulability can be maintained is about 200°C at the most. Therefore, it has been impossible to employ such an organic insulated coated wire for application for which guarantee for insulability is required under a high temperature of at least 200°C.

Further, the insulated wire which is improved in heat resistance through an insulator tube of ceramics has disadvantages such as inferior flexibility. The MI cable is formed by a heat resistant alloy tube and a conductor, and hence the outer diameter of the cable is increased with respect to the conductor radius. Thus, the MI cable has a relatively large section with respect to electric energy allowed by the conductor which is passed through the heat resistant alloy tube. In order to use the MI cable as a wire for winding which is wound on a bobbin etc. in the form of a coil, however, it is necessary to bend the heat resistant alloy tube in prescribed curvature. In this case, bending performed on the heat resistant alloy tube involves difficulty. When the MI cable is wound in the form of a coil, further, it is difficult to improve space factor since the tube of its outer layer is thick as compared with the conductor.

Further, when the fiber-glass braided insulated wire having heat resistance is employed and worked into a prescribed configuration in response to its application, the network of the braid is disturbed to cause a breakdown. In addition, dust of glass is generated from the glass fiber. This glass dust may serve as a gas adsorption source. Therefore, when the fiber-glass braided insulated wire is used under environment for which a high degree of vacuum is required, it has been impossible to maintain a high degree of vacuum due to the gas adsorption source provided by the glass dust.

On the other hand, there has generally been the so-called alumite wire prepared by performing anodic oxidation treatment on a wire of aluminum or an aluminum alloy, as an insulated wire which is excellent in heat resistance, insulability and heat dissipativity. In this alumite wire, its base material is restricted to aluminum. Further, an inorganic insulating layer formed on the base material is also restricted to aluminum oxide. Thus, there has been such a problem that it is impossible to select combinations of the base material and the inorganic insulating layer which are suitable for various uses. EP-A-0 292 780 describes an electric wire with a coating of a gel film on a conductor. EP-A-188 369 describes an insulation with a Keying layer of oxide, such as Al₂O₃, SiO₂, TiO₂ and TaO₂.

### Disclosure of the Invention

Accordingly, the present invention has been proposed in order to solve the aforementioned problems, and its object is to provide an insulated wire comprising the following items:
(a) It has high insulability under environment of a high temperature.
(b) It is excellent in flexibility.
(c) It comprises no gas adsorption source.
(d) Combinations of a base material and an inorganic insulating layer suitable for various uses can be selected.

An insulated wire according to the present invention comprises a base material, a chromium oxide containing layer, and an oxide insulating layer. The base material has an outer surface, and includes a conductor. The chromium oxide containing layer is formed on the outer surface of the base material. The oxide insulating layer is formed by applying a precursor solution of a metallic oxide onto the chromium oxide containing layer by a sol-gel method or an organic acid salt pyrolytic method.

The chromium oxide containing layer is preferably formed by an electrochemical technique. The electrochemical technique includes electrolytic plating or electroless plating. The underlayer to be provided with the oxide insulating layer may be a CrO₃₋ₓ (1.5 ≦ X ≦ 2.5) layer, in order to preferably serve as an adhesion layer. Namely, the layer formed by the electrochemical technique has a chromium oxide layer as its outermost layer. The oxide insulating layer preferably contains silicon oxide, aluminum oxide or zirconium oxide. As to the base material, copper or a copper alloy is preferably employed in view of high conductivity and the cost. In consideration of a use at a higher temperature or the like, nickel chromium, silver, iron or a ferroalloy, a stainless steel alloy, or titanium or a titanium alloy is preferably contained in the surface layer of the base material.

It is known that a chrome plated layer is formed on a conductor of copper or a copper alloy etc. as an excellent adhesion layer. However, insulating oxide ceramics such as silicon oxide obtained by heat treatment of a precursor solution of a metallic oxide hardly exhibits adhesion with respect to the chrome plated layer. This is based on recognition of the inventors.

In an insulated wire obtained by directly forming a thin film of ceramics on a surface of a conductor made of copper, further, the ceramics thin film serving as an insulating layer has insufficient adhesion with respect to a base material.

According to the present invention, therefore, a layer having a chromium oxide layer as its outermost layer is formed on an outer surface of a base material. Insulating oxide ceramics adheres onto the chromium oxide layer as a layer having excellent adhesion.

The aforementioned chromium oxide layer is formed by an electrochemical technique. When the chromium oxide layer is formed by electrolytic plating, a substance obtained by adding a small amount of organic acid to an aqueous solution of chromic anhydride is used as an electrolyte. Although a sergeant bath mainly composed of chromic anhydride or sulfuric acid is known as an electrolytic bath employed for chrome plating, it is different from this bath in the following point: Namely, mineral acid mixed into the electrolytic bath has a function of dissolving chromic anhydride which is generated on the surface of a plated layer in electrolytic plating. Therefore, a glossy metallic chrome layer is plated when a sergeant bath is employed. In the present invention, it is necessary to preferentially plate chromium oxide. Therefore, a small amount of organic acid is added to an electrolytic bath employed in the present invention. In a case of using mineral acid such as sulfuric acid, further, it is necessary to employ a particularly dilute electrolytic bath. Namely, chromic anhydride concentration is not more than 50 g/ℓ and sulfuric acid concentration is not more than 1 g/ℓ. Further, while a thin film of insulating ceramics is formed on the outer surface of a layer mainly composed of chromium oxide by heat treatment of a precursor solution of a metallic oxide, the layer mainly composed of chromium oxide preferably has a roughened surface, in order to further increase adhesion of the thin film.

The chromium oxide containing layer may be formed by electrolytic plating employing an electrolyte which is prepared by adding sodium citrate, sodium carbonate or the like, for example, to an aqueous solution of sodium chromate. In this case, the as-formed layer is mainly composed of chromium oxide, which is generated by trivalent reduction of hexavalent chromium contained in the electrolyte. If copper is used as a base material in this electrolytic plating treatment, the base material surface is oxidized and the chromium oxide containing layer is formed in the exterior thereof. However, adhesion of the chromium oxide containing layer with respect to the base material is not reduced by such oxidation of the base material surface.

Conditions for electrolytic plating for forming the inventive chromium oxide containing layer are different from those for general bright plating in treatment current density etc. Although the current density is set at 10 to 60 A/dm² in the bright plating, depending on the treatment temperature, the current density is set at 100 to 200 A/dm² in the present invention. A chromium oxide containing layer having a roughened surface can be formed by this condition of the current density.

On the chromium oxide containing layer, an insulating oxide layer is formed by application of a precursor solution of a metallic oxide. The precursor solution of a metallic oxide mentioned in this specification is a solution prepared from a metal organic compound, which is broadly classified in correspondence to a sol-gel method or an organic acid salt pyrolytic method, and those of the following two types are included:

The first type of precursor solution is a solution which is generated by making hydrolytic reaction and dehydration/condensation reaction of a compound containing hydrolyzable metal-oxygen-organic group bonds such as metal alkoxide or acetate of a metal. This solution may contain an organic solvent such as alcohol, a raw material compound such as metal alkoxide, and water and a catalyst required for hydrolytic reaction. Further, it generally contains an organic residual group such as alkoxide, dissimilarly to hydroxide sol that is generated from inorganic salt.

The second type of precursor solution is a solution prepared by dissolving a metal organic compound such as organic acid salt of a metal in an appropriate organic solvent. In a method employing this type of precursor solution, a metallic oxide is generated by pyrolyzation through heating after application. Therefore, a decomposition temperature of the employed metal organic compound must be lower than its boiling point or sublimation point.

The metal organic compound mentioned in this specification is a concept similar to "metal-organic compounds" described in Journal of Materials Science 12 (1977) pp. 1203 to 1208, for example.

Further, the applied layer must be left at a temperature higher than the room temperature, for volatilization of the organic solvent and removal of a residual organic substance. However, the temperature of the atmosphere for such leaving must not be higher than the melting point of the metal forming the base material.

It is possible to form almost all metallic oxide-based ceramics covering by application of a precursor solution of a metallic oxide. SiO₂, Al₂O₃, ZrO₄, TiO₂, MgO or the like can be listed as an example of a metallic oxide formed by this method. Further, ethoxide, propoxide, butoxide or the like can be listed as metal alkoxide employed for the first type of precursor solution. Metallic salt such as naphtanic acid, caprylic acid, stearic acid, octylic acid or the like is preferable as organic salt employed for the second type of precursor solution.

The oxide insulating layer formed from the precursor solution of the metallic oxide by the sol-gel method or the organic acid salt pyrolytic method is an oxide which is completely converted to a metallic oxide. This oxide is preferably formed by heat treatment under an atmosphere in an oxygen current. In general, decomposition of the compound contained in the solution which is applied onto the chromium oxide containing layer is completely terminated at a temperature of about 500°C. If the same is heat treated at a higher temperature, however, reaction between elements forming the chromium oxide containing layer and a metal or semimetal contained in the applied solution is facilitated, whereby adhesion between the chromium oxide containing layer and the oxide layer is improved.

Thus, the oxide insulating layer converted to ceramics exhibits excellent heat resistance/insulability also under a high temperature of at least 500°C. Further, the chromium oxide containing layer is excellent in adhesion to the conductor forming the base material. Therefore, adhesion between the oxide insulating layer and the outer surface of the base material is improved as compared with the case of directly forming the oxide insulating layer on the outer surface of the conductor by heat treatment of the precursor solution of the metallic oxide. Thus, the insulated wire provided according to the present invention has heat resistance/insulability, as well as excellent flexibility.

Further, the oxide insulating layer formed on the chromium oxide containing layer has a smooth outer surface. Therefore, a high breakdown voltage proportionate to the film thickness can be obtained, while it is possible to reduce a gas adsorption source.

According to the present invention, in addition, the chromium oxide containing layer is formed between the base material and the oxide insulating layer. Therefore, combinations with the inorganic insulating layer suitable for various uses can be selected through the chromium oxide containing layer.

### Brief Description of the Drawings

Fig. 1 is a sectional view showing a cross section of an insulated wire according to the present invention in correspondence to Example 1.

Fig. 2 is a sectional view showing a cross section of an insulated wire according to the present invention in correspondence to Example 2.

Fig. 3 is a sectional view showing a cross section of an insulated wire according to the present invention in correspondence to Example 3.

Fig. 4 is a sectional view showing a cross section of an insulated wire according to the present invention in correspondence to Example 4.

Fig. 5 is a graph showing the result of measurement of surface roughness of a chromium oxide containing layer formed in accordance with Example 3 or Example 4.

Fig. 6 is a graph showing the result of measurement of surface roughness of a chrome plated layer formed in accordance with Reference Example.

### Best Modes of Carrying Out the Invention

### Example 1

### (a) Formation of Chromium Oxide Containing Layer

Electrolytic plating treatment was performed on an outer surface of a copper wire of 2 mmφ in wire diameter. At this time, an electrolyte was prepared from that having concentration of 40 g/ℓ of chromic anhydride and 0.45 g/ℓ of sulfuric acid. As to plating conditions, the bath temperature was 50°C, the current density was 140 A/dm², and the treatment time was two minutes. Thus, a chromium oxide containing layer was formed on the outer surface of the copper wire with a film thickness of about 1 µm.

### (b) Preparation of Coating Solution used for Sol-Gel Method

Nitric acid was added to a solution mixed in mole ratios of tetrabutyl orthosilicate:water:isopropyl alcohol = 8:32:60 in a ratio of 3/100 mole with respect to tetrabutyl orthosilicate. Thereafter this solution was heated/stirred at a temperature of 80°C for two hours. Thus, a coating solution used for a sol-gel method was synthesized.

### (c) Coating

The wire obtained by (a) was dipped in the coating solution of (b). A step of heating at a temperature of 400°C for 10 minutes was performed ten times on the wire whose outer surface was thus coated with the coating solution. Finally, this wire was heated in an oxygen current of 500°C in temperature for 10 minutes.

An insulated covered wire obtained in the aforementioned manner is shown in Fig. 1. Fig. 1 is a sectional view showing a cross section of the insulated wire obtained according to Example 1. Referring to Fig. 1, a chromium oxide containing layer 2 is formed on an outer surface of a copper wire 1. On this chromium oxide containing layer 2, a silicon oxide layer 3 is formed by the sol-gel method as an oxide insulating layer. The film thickness of an insulating layer formed by the chromium oxide containing layer 2 and the silicon oxide layer 3 was about 4.0 µm.

A breakdown voltage was measured in order to evaluate insulability of the obtained insulated wire. Its breakdown voltage was 800 V under the room temperature, and was 600 V under a temperature of 800°C. Even if this insulated wire was wound on an outer peripheral surface of a cylinder having a diameter of 10 cm, no cracking was caused in the insulating layer.

### Example 2

### (a) Formation of Chromium Oxide Containing Layer

A copper wire of 2 mmφ in wire diameter was vapor-degreased through use of perchloroethylene. Thereafter the copper wire was dipped in a solution mixed in volume ratios of 85 % phosphoric acid:70 % nitric acid:water = 15:2:3, thereby roughening its surface.

Then, the copper wire was used as a cathode and a stainless steel plate was used as an anode to perform electrolytic plating treatment by feeding a direct current of 0.05 A/dm². At this time, a solution of about 1ℓ prepared by dissolving 30 g of sodium chromate, 30 g of sodium citrate and 30 g of sodium carbonate in water respectively was used as an electrolyte.

Thus, a copper oxide layer having a film thickness of about 1 µm was formed on the outer surface of the copper wire, and a chromium oxide containing layer was formed in its exterior with a film thickness of about 0.1 µm.

### (b) Preparation of Coating Solution used for Sol-Gel Method

A solution mixed in mole ratios of tetrabutyl orthozirconate [(C₄H₉O)₄Zr]:water:n-butyl alcohol = 5:15:80 was heated/stirred at a temperature of 120°C for two hours. Thus, a coating solution used for a sol-gel method was synthesized.

### (c) Coating

The wire obtained by (a) was dipped in the coating solution of (b). A step of heating at a temperature of 400°C for 10 minutes was performed ten times on the wire whose outer surface was thus coated with the coating solution.

An insulated covered wire obtained in the aforementioned manner is shown in Fig. 2. Fig. 2 is a sectional view showing a cross section of the insulated wire obtained according to Example 2. Referring to Fig. 2, a copper oxide layer 12 is formed on the outer surface of a copper wire 11. Further, a chromium oxide containing layer 13 is formed in the exterior of this copper oxide layer 12. On this chromium oxide containing layer 13, a zirconium oxide layer 14 is formed by the sol-gel method as an oxide insulating layer. The film thickness of an insulating layer formed by the copper oxide layer 12, the chromium oxide containing layer 13 and the zirconium oxide layer 14 was about 3.0 µm.

A breakdown voltage was measured in order to evaluate insulability of the obtained insulated wire. Its breakdown voltage was 700 V under the room temperature, and was 500 V under a temperature of 700°C. Even if this insulated wire was wound on an outer peripheral surface of a cylinder having a diameter of 10 cm, no cracking was caused in the insulating layer.

### Example 3

### (a) Formation of Chromium Oxide Containing Layer

Electrolytic plating treatment was performed on an outer surface of a nickel-plated copper wire of 1.8 mmφ in wire diameter. At this time, an electrolyte was prepared from that having concentration of 200 g/ℓ of chromic anhydride, 20 g/ℓ of ammonium methavanadate and 6.5 g/ℓ of acetic acid. As to plating conditions, the base material was used as a cathode, while the bath temperature was 50°C, the current density was 150 A/dm², and the treatment time was two minutes. Thus, a chromium oxide containing layer was formed on the outer surface of the nickel-plated copper wire with a film thickness of about 1 µm.

As to the surface state of the chromium oxide containing layer, the center line average roughness Ra was 0.15 µm and the maximum height Ry was 0.87 µm in accordance with Surface Roughness of ISO468-1982. The surface roughness was measured by using a surface contour measurer DEKTAK3030 made by Sloan Inc., U.S.A., under conditions of a tracer diameter of 0.5 µm, a stylus pressure of 10 mg, a reference length of 50 µm, and no use of a cutoff filter. The result of measurement is shown in Fig. 5.

### (b) Preparation of Coating Solution used for Organic Acid Salt Pyrolytic Method

A coating solution was prepared by dissolving 20 g of 2-ethyl-hexanoic silicate in 100 mℓ of dibutyl ether.

### (c) The wire obtained by (a) was dipped in the coating solution of (b). A step of heating at a temperature of 500°C for 10 minutes was performed ten times on the wire whose outer surface was thus coated with the coating solution.

An insulated covered wire obtained in the aforementioned manner is shown in Fig. 3. Fig. 3 is a sectional view showing a cross section of the insulated wire obtained according to Example 3. Referring to Fig. 3, a nickel-plated copper wire comprising a nickel-plated layer 22 formed on an outer surface of a copper wire 21 is used as a base material. A chromium oxide containing layer 23 is formed on the outer surface of this nickel-plated copper wire. On the chromium oxide containing layer 23, a silicon oxide layer 24 is formed by an organic acid salt pyrolytic method as an oxide insulating layer. The film thickness of an insulating layer formed by the chromium oxide containing layer 23 and the silicon oxide layer 24 was about 5 µm.

A breakdown voltage was measured in order to evaluate insulability of the obtained insulated wire. The breakdown voltage was 500 V under the room temperature, and was 300 V under a temperature of 800°C. Even if this insulated wire was wound on an outer peripheral surface of a cylinder having a diameter of 5 cm, no cracking was caused in the insulating layer.

### Example 4

### (a) Formation of Chromium Oxide Containing Layer

The so-called stainless steel clad copper wire of 1.8 mmφ in wire diameter, in which a stainless steel alloy (SUS304) was engaged on an outer surface of a copper wire, was used as a base material. Electrolytic plating treatment was performed on the outer surface of this stainless steel clad copper wire. At this time, an electrolyte was prepared from that having concentration of 200 g/ℓ of chromic anhydride, 20 g/ℓ of ammonium methavanadate and 6.5 g/ℓ of acetic acid. As to plating conditions, the base material was used as a cathode, while the bath temperature was 50°C, the current density was 150 A/dm² and the treatment temperature was two minutes. Thus, a chromium oxide containing layer was formed on the outer surface of the stainless steel clad copper wire with a film thickness of about 1 µm.

As to its surface state, the center line average roughness Ra was 0.15 µm, and the maximum height Ry was 0.87 µm in accordance with Surface Roughness of ISO468-1982. The measurement was performed by using a surface contour measurer DEXTAK3030 made by Sloan Inc., U.S.A., under conditions of a tracer diameter of 0.5 µm, a stylus pressure of 10 mg, a reference length of 50 µm, and no use of a cutoff filter. As the result of this measurement, that shown in Fig. 5 was obtained similarly to Example 3.

### (b) Preparation of Coating Solution used for Organic Acid Salt Pyrolytic Method

25 g of aluminum tetra-i-butoxide was dissolved in 100 mℓ of diethylene glycol monomethyl ether, and thereafter heated/stirred at 150°C for one hour. This solution was stood to be cooled to the room temperature, and thereafter mixed with 3 g of alumina particles of 0.03 µm in nominal particle size, thereby preparing a coating solution.

### (c) Coating

The wire obtained by (a) was dipped in the coating solution of (b). A step of heating at a temperature of 500°C for 10 minutes was performed ten times on the wire whose outer surface was thus coated with the coating solution.

An insulated covered wire obtained in the aforementioned manner is shown in Fig. 4. Fig. 4 is a sectional view showing a cross section of the insulated wire obtained according to Example 4. Referring to Fig. 4, a stainless steel clad copper wire having a stainless steel alloy layer 32 on an outer surface of a copper wire 31 is used as a base material. A chromium oxide containing layer 33 is formed on the outer surface of the stainless steel clad copper wire. On this chromium oxide containing layer 33, an aluminum oxide layer 34 is formed by an organic acid salt pyrolytic method as an oxide insulating layer. This aluminum oxide layer 34 consists of an aluminum oxide mixed layer containing aluminum particulates which have been mixed in the coating solution from the start. The film thickness of an insulating layer formed by the chromium oxide containing layer 33 and the aluminum oxide layer 34 was about 12 µm.

A breakdown voltage was measured in order to evaluate insulability of the obtained insulated wire. Its breakdown voltage was 900 V under the room temperature, and was 700 V under a temperature of 800°C. Even if this insulated wire was wound on an outer peripheral surface of a cylinder having a diameter of 15 cm, no cracking was caused in the insulating layer.

### Reference Example

### (a) Formation of Metallic Chrome Plated Layer

Electrolytic plating treatment was performed on an outer surface of a nickel-plated copper wire of 1.8 mmφ in wire diameter. At this time, an electrolyte to be used was prepared from that having concentration of 250 g/ℓ of chromic anhydride and 2.5 g/ℓ of sulfuric acid. As to plating conditions, the base material was used as a cathode, while the bath temperature was 50°C, the current density was 40 A/dm², and the treatment time was two minutes. Thus, a chrome containing layer was formed on the outer surface of the nickel-plated copper wire with a film thickness of about 1 µm.

As to its surface state, the center line average roughness Ra was 0.06 µm and the maximum height Ry was 0.51 µm in accordance with Surface Roughness of ISO468-1982. The measurement was performed by using a surface contour measurer DEKTAK3030 made by Sloan Inc., U.S.A., under conditions of a tracer diameter of 0.5 µm, a stylus pressure of 10 mg, a reference length of 50 µm, and no use of a cutoff filter. The result of this measurement is shown in Fig. 6. A glossy metallic chrome layer was formed on the outer surface of the nickel-plated copper wire.

### (b) Preparation of Coating Solution used for Organic Acid Salt Pyrolytic Method

A coating solution was prepared by dissolving 20 g of 2-ethyl-hexanoic silicate in 100 mℓ of dibutyl ether.

### (c) Coating

The wire obtained by (a) was dipped in the coating solution of (b). A step of heating at a temperature of 500°C for 10 minutes was performed on the wire whose outer surface was thus coated with the coating solution, whereby the as-formed insulating layer was separated like a film after heating, and exhibited no adhesion.

### Industrial Availability

As hereinabove described, the insulated wire according to the present invention is suitable for a distribution wire, a wire for winding or the like, which is employed under high-vacuum environment or high-temperature environment such as a high vacuum apparatus or a high temperature service apparatus.

## Claims

1. An insulated wire comprising:
a base material (1) having an outer surface and including an electrical conductor,
a chromium oxide containing layer (2) formed on the outer surface of said base material, and
an oxide insulating layer (3) formed by applying a precursor solution of a metallic oxide onto said chromium oxide containing layer.

2. An insulated wire in accordance with claim 1, wherein said chromium oxide containing layer (2) is formed by electrolytic plating.

3. An insulated wire in accordance with claim 1, wherein said oxide insulating layer (3) contains any one of silicon oxide, aluminum oxide and zirconium oxide.

4. An insulated wire in accordance with claim 1, wherein said base material (1) contains either copper or a copper alloy.

5. An insulated wire in accordance with claim 4, wherein said base material contains any one of nickel, chromium and a stainless steel alloy in its surface layer (22).

6. An insulated wire in accordance with claim 1, wherein said oxide insulating layer (3) contains ceramics particulates dispersed therein.

7. An insulated wire comprising:
A base material (1) having an outer surface and including an electrical conductor,
a chromium oxide containing layer (2) formed on the outer surface of said base material, and
an oxide insulating layer (3) formed on said chromium oxide containing layer by a sol-gel method.

8. An insulated wire comprising:
a base material (21) having an outer surface and including an electrical conductor,
a chromium oxide containing layer (23,33) formed on the outer surface of said base material, and
an oxide insulating layer (24,34) formed on said chromium oxide containing layer by an organic acid salt pyrolytic method.

## Patentansprüche

1. Isolierte Litze umfassend:
- ein Grundmaterial (1), die eine äußere Fläche aufweist und einen elektrischen Leiter umfaßt,
- eine chromoxidhaltige Schicht (2), die an der äußeren Fläche des Grundmaterials gebildet ist und
- eine isolierende Oxid-Schicht (3), welche durch Anwenden einer Vorstufelösung eines Metalloxides auf der chromoxidhaltigen Schicht gebildet wird.

2. Isolierende Litze nach Anspruch 1, worin die chromoxidhaltige Schicht (2) durch Electrolyt-Plattierung gebildet ist.

3. Isolierende Litze nach Anspruch 1, worin die isolierende Oxidschicht (3) ein beliebiges der Materialien Siliziumoxid, Aluminiumoxid und Zirkoniumoxid enthält.

4. Isolierende Litze nach Anspruch 1, worin das Grundmaterial (1) entweder Kupfer oder eine Kupferlegierung enthält.

5. Isolierende Litze nach Anspruch 4, worin das Grundmaterial ein beliebiges der Materialien Nickel, Chrom und rostfreie Stahllegierung in ihrer Oberflächenschicht (22) enthält.

6. Isolierende Litze nach Anspruch 1, worin die isolierende Oxidschicht (3) darin dispergierte Keramikteilchen enthält.

7. Isolierende Litze umfassend:
- ein Grundmaterial (1), das eine äußere Fläche aufweist und einen elektrischen Leiter umfaßt,
- eine chromoxidhaltige Schicht (2), die an der äußeren Fläche des Grundmaterials vorgesehen ist, und
- eine isolierende Oxidschicht (3), welche auf der chromoxidhaltigen Schicht durch ein Sol-Gel-Verfahren gebildet ist.

8. Isolierende Litze umfassend:
- ein Grundmaterial (1), das eine äußere Fläche aufweist und einen elektrischen Leiter umfaßt,
- eine chromoxidhaltige Schicht (2), die an der äußeren Fläche des Grundmaterials vorgesehen ist und
- eine isolierende Oxidschicht (3), welche auf der chromoxidhaltigen Schicht durch ein pyrolytisches Verfahren mit Salz einer organischen Säure gebildet ist.

## Revendications

1. Fil électrique isolé comprenant :
un matériau de base (1) comportant une surface extérieure et incorporant un conducteur électrique,
une couche contenant de l'oxyde de chrome (2) formée sur la surface extérieure du matériau de base, et
une couche isolante d'oxyde (3) formée par application d'une solution de précurseur d'un oxyde métallique sur la couche contenant l'oxyde de chrome.

2. Fil électrique isolé selon la revendication 1, dans lequel la couche (2) contenant l'oxyde de chrome est formée par plaquage électrolytique.

3. Fil électrique isolé selon la revendication 1, dans lequel la couche isolante d'oxyde (3) contient l'un quelconque parmi l'oxyde de silicium, l'oxyde d'aluminium et l'oxyde de zirconium.

4. Fil électrique isolé selon la revendication 1, dans lequel le matériau de base (1) contient soit du cuivre soit un alliage de cuivre.

5. Fil électrique isolé selon la revendication 4, dans lequel le matériau de base contient l'un quelconque du nickel, du chrome et un alliage en acier inoxydable dans sa couche de surface (22).

6. Fil électrique isolé selon la revendication 1, dans lequel la couche isolante d'oxyde (3) contient des particules de céramique dispersées dans celle-ci.

7. Fil électrique isolé comprenant :
un matériau de base (1) comportant une surface extérieure et incorporant un conducteur électrique,
une couche (2) contenant de l'oxyde de chrome, formée sur la surface extérieure du matériau de base, et
une couche isolante d'oxyde (3), formée sur la couche contenant l'oxyde de chrome par un procédé sol-gel.

8. Fil électrique isolé comprenant :
un matériau de base (21) comportant une surface extérieure et incorporant un conducteur électrique,
une couche (23, 33) contenant un oxyde de chrome, formée sur la surface extérieure du matériau de base, et
une couche isolante d'oxyde (24, 34) formée sur la couche contenant l'oxyde de chrome par un procédé pyrolytique au sel d'un acide organique.
